

Jan. 10, 1939.

F. M. CLARK

2,143,685

ELECTRIC DEVICE AND DIELECTRIC MATERIALS THEREFOR

Filed May 25, 1935

Fig. 1.



Fig. 2.



Fig. 3.



Fig. 4.



Inventor:  
Frank M. Clark,  
by *Harry E. Dunham*  
His Attorney.

## UNITED STATES PATENT OFFICE

2,143,685

ELECTRIC DEVICE AND DIELECTRIC  
MATERIALS THEREFORFrank M. Clark, Pittsfield, Mass., assignor to  
General Electric Company, a corporation of  
New York

Application May 25, 1935, Serial No. 23,404

9 Claims. (CL. 252—1)

The present invention comprises a liquid dielectric and electrically insulating material.

In my prior Patent 1,931,455, patented October 17, 1933, I have described various non-inflammable dielectric and insulating compositions which consist of one or more aromatic hydrocarbons containing combined chlorine, or other suitable halogen. When such halogenated material is decomposed, which may be the case when an electric arc strikes therethrough, as in a circuit breaker, then hydrogen halide gas is formed. In the presence of water vapor, which may be of atmospheric origin, some gaseous hydrogen halide tends to remain in the electrical apparatus as a fog. In some cases such halide and water may become emulsified in the halogenated hydrocarbon where it may cause corrosion of metal parts or otherwise may harmfully affect the apparatus. While the halogen hydride gas may be removed by an external chemical absorber, as described in my prior U. S. Patent 1,964,684, patented June 26, 1934, its presence is in any event a source of difficulty.

In accordance with my present invention I have provided new liquid compositions comprising as a preponderant ingredient one or more halogenated nitrile carbon compounds, and electric devices containing such compositions as insulating and heat transfer agents. By the term "nitriles" I include those materials in which one carbon atom combined with either an alkyl or an aryl group is combined with nitrogen, the general formula being  $RC:N$ .

The general or empirical formula for the halogenated nitriles is  $RX_nC:N$  in which R represents an aromatic radical, or an aromatic derivative of an alkyl radical (as in the benzyl compounds), in which compound hydrogen atoms have been displaced by halogen (X) to an extent (n) preferably affording a chemical equivalency of hydrogen and halogen in the total mixture. Such materials are non-inflammable and possess the property of absorbing hydrogen halide which has been freed from its parent molecule by decomposition.

The accompanying drawing illustrates somewhat conventionally different forms of electrical device in which compositions embodying my present invention may be employed for dielectric and insulating purposes. Fig. 1 is a side elevation partly in section of a transformer; Fig. 2 similarly illustrates a switch; Fig. 3 diagrammatically illustrates a capacitor; and Fig. 4 is a side view of a short section of cable the casing

being shown in part removed to permit interior parts to be seen.

Among the compounds representative of the different classes of hydrocarbon compounds included in the term "nitriles" are the aromatic nitriles as benzonitrile and tolunitrile and phenylated aliphatic nitriles, as benzyl cyanide.

I prefer to employ either a halogenated phenyl nitrile compound, such, for example, as chlorinated benzonitrile, or chlorinated tolunitrile, or a halogenated phenylated aliphatic nitrile compound, such, for example, as chlorinated benzyl nitrile or tolylacetone nitrile. In general halogenated aromatic nitrile compounds should be chosen in which the halogen content equals, or exceeds, the hydrogen content in order to insure non-inflammability.

The halogenated nitrile compounds which are employed for the purpose of my invention need not be chemically pure material. The halogenated aromatic nitrile compositions most suitable for my invention are mixtures of halogenated nitrile isomers. Such isomeric mixtures have a desired property of remaining liquid down to low temperature which, as explained in my prior patents, is a highly desirable property in liquid dielectrics for high potential apparatus.

In the following example of the preparation of a nitrile dielectric composition, the halogen element is represented by chlorine. Other halogens may be substituted for chlorine without departing from my invention. Chlorinated benzyl cyanide,  $PhCl_nCH_2CN$  (n being 1, 2, 3, 4 or 5), may be made by the chemical interaction of a chlorinated benzyl chloride, an alcohol and a cyanide. In the preparation of a trichlor benzyl cyanide composition the following mixture is heated to a reaction temperature, preferably while being agitated:

|                                                       | Parts by weight |
|-------------------------------------------------------|-----------------|
| Technical mixture of trichlor benzyl chloride isomers | 40              |
| Ethyl alcohol                                         | 50              |
| Potassium cyanide                                     | 13              |
| Water                                                 | 12 45           |

The reaction requires about twelve hours. The product, which is a mixture of isomers of trichlor benzyl cyanide, is subjected to distillation followed by washing to remove undesired contaminants and in general is purified by well-known refining methods.

Chlorinated benzyl chloride can be obtained from toluene,  $C_6H_5CH_3$  by chlorination: first, introducing chlorine in the phenyl or ring part of

the toluene in the presence of an iron catalyst at temperatures of the order of 25 to 50° C., and second, the  $\text{CH}_3$  side chain may be chlorinated in the presence of sulphur at a higher temperature, ordinarily at 140 to 150° C.

The product obtained, when a technical mixture of the isomers of trichlorbenzyl chloride is used, is a clear liquid having a specific gravity at 15.5° C. (referred to water at the same temperature) of 1.53 and boiling in the range of 185 to 215° C. at a pressure of about 25 millimeters of mercury. Its refractive index at 25° C. is 1.5850. Its electrical resistivity is higher than  $1 \times 10^{10}$  ohms per cm. cubed. The dielectric constant is high, being in the neighborhood of 20. It has a pour point of about minus 30° C. (determined by A. S. T. M. test procedure D97—27T) and a viscosity of about 47 seconds at 37.8° C. Saybolt Universal.

Tetrachlor benzyl cyanide may be prepared as a mixture of its isomers by a similar method to that already described for the preparation of the trichlor benzyl cyanide. In this case, however, the chlorination of the toluene at 25 to 50° C. in the presence of an iron catalyst is carried to such degree that four chlorine atoms are introduced into the phenyl or ring structure of the toluene molecule.

Tetrachlor benzyl cyanide as a mixture of its isomers is a more viscous liquid of higher pour point than the trichlor compound. It boils at 25 millimeters pressure within the range of 220 to 250° C., has a specific gravity (15.5°/15.5° C.) of 1.58, a viscosity at 37.8° C. of 160 seconds, Saybolt Universal, a pour point (A. S. T. M.) of minus 5° C. and a refractive index of 1.598.

The phenyl nitrile compounds may be compounded or mixed with one or more other liquid dielectric materials, such for example as chlorinated diphenyl, chlorinated diphenyl oxide, chlorinated naphthalene, or other chlorinated polyphenyls, chlorinated benzene and chlorinated polyphenyls containing an alkyl group, such as chlorinated diphenyl methane, thereby producing mixtures having a viscosity best suited for particular purposes.

Chlorinated diphenyl of 60% chlorine content is extremely viscous at room temperature, having a pour point of about 30° C. (A. S. T. M. standard), and, therefore, being capable of use only with difficulty for impregnating capacitors or other devices. Mixtures may be prepared comprising this material and a nitrile such as trichlor benzyl cyanide, the product having pour points and viscosities as indicated below, the indicated proportions being by weight:

|    | Per cent chlor<br>diphenyl (60%<br>chlorine<br>content) | Per cent<br>trichlor<br>benzyl<br>cyanide | Pour<br>point | Viscosity<br>Saybolt at<br>37.8° C. |
|----|---------------------------------------------------------|-------------------------------------------|---------------|-------------------------------------|
|    |                                                         |                                           |               | ° C.<br>Plus 2                      |
| 60 | 75                                                      | 25                                        | 740           |                                     |
| 65 | 50                                                      | 50                                        | 123           |                                     |
|    | 25                                                      | 75                                        | 65            | Minus 27                            |

Such mixtures when having pour points below 0° C. are suitable for uses requiring a fluid material, for example, as dielectric and insulating materials in electric devices, such as transformers, capacitors, cables, switches, fuses, and the like.

The outstanding useful property of nitrile compounds here under consideration is their affinity for hydrogen chloride, no solid precipitate being formed and no deleterious or poisonous gases

being evolved. The hydrogen chloride gas formed from the chlorinated benzyl cyanide component of the above composition when decomposed by the electric arc is absorbed by the body of undecomposed cyanide. A harmless addition product is formed which dissolves in the benzyl cyanide.

In U. S. Patent No. 2,105,406 for Liquid insulating composition, patented January 11, 1938, I have described and claimed insulating and cooling compositions consisting of halogenated hydrocarbons, or mixtures thereof, and containing a fixative which may consist of halogenated nitrile whereby the evolution of hydrogen chloride from such compositions is inhibited.

Dielectric compositions consisting preponderantly of a halogenated nitrile may be used in various electrical devices of which four have been shown as illustrative. The transformer shown in Fig. 1 comprises a tank 1, containing a magnetic core 2, and transformer windings 3, the latter being surrounded by a liquid halogenated nitrile composition 4. Only one high tension terminal 5 of the transformer windings is visible in the drawing. While the drawing shows also a pressure release conduit 6, such conduit is separated from the main tank 7 by a diaphragm 8 which will only be ruptured under such extraordinary circumstances in which the decomposition of the liquid 4 exceeds the gas-absorbing capability of the fixative in the composition. A solid gas-absorber 9 may be provided in the conduit 6 but ordinarily will not be necessary. No gas release conduit has been shown for the circuit breaker of Fig. 2, which comprises a tank 11, fixed contacts 12, 13, and cooperating movable contacts 14, 15. The latter are mounted on a support 16 which in turn is operatively connected to actuating levers 17. The liquid arc-quenching material 18 embodies the present invention. The capacitor indicated in Fig. 3 comprises armatures or plates 20, 21 and an interposed porous dielectric layer 22 which may consist of paper. The layer 22 is impregnated by a composition made as herein described.

It has been found that capacitors having aluminum foil armatures and kraft paper spacers when impregnated with trichlor benzyl cyanide have a capacity of one microfarad for 2.28 square feet of electrode surface, whereas similar capacitors impregnated with chlorinated diphenyl require approximately 5 square feet of electrode surface for one microfarad capacity and similar capacitors impregnated with mineral oil require seven square feet of surface for one microfarad capacity. The cable of Fig. 4 comprises a core 24, cable conductors 25, insulation 26, which may consist of paper and an external casing 27. The space between the insulated conductors 25 and the casing may contain a liquid composition embodying my present invention.

What I claim as new and desire to secure by Letters Patent of the United States, is:

1. In an electric device an insulating composition consisting essentially of a mixture of isomers of liquid chlorinated benzyl nitrile containing at least three combined chlorine atoms per molecule.

2. An electric device containing an insulating and heat transfer medium consisting essentially of a mixture of isomers of hydrocarbon compounds having the chemical formula  $\text{RX}_n\text{CN}$  (R being an aromatic radical or an aromatic derivative of an alkyl radical, X being a halogen, n being equal to 3 or more, C being carbon, and N being nitrogen), said material being liquid,

- non-combustible, and being capable of absorbing hydrogen halide without forming precipitates.
3. In an electric device, an insulating composition of matter consisting of a liquid mixture of isomers of chlorinated phenyl nitrile, said mixture containing sufficient chlorine to be non-combustible, evolving non-combustible gas upon decomposition by an electric arc, and being capable of absorbing hydrogen chloride.
- 10 4. In an electric device, a dielectric and insulating composition consisting essentially of a liquid mixture of a plurality of chlorinated benzyl cyanide isomers, said mixture being non-combustible and being capable of absorbing hydrogen chloride.
- 15 5. In an electric device, a dielectric composition consisting essentially of a liquid mixture of isomers of trichlor benzyl cyanide.
6. In an electric device, a dielectric composition consisting essentially of a liquid mixture of isomers of tetrachlor benzyl cyanide.
- 20 7. A dielectric and insulating composition consisting essentially of a liquid mixture of isomers of trichlor benzyl cyanide having a pour point of about  $-30^{\circ}$  C., a viscosity of about 47 seconds at  $37.8^{\circ}$  C., and boiling in the range of about 185 to  $215^{\circ}$  C., at a pressure of about 25 mm. of mercury.
8. A dielectric and insulating composition consisting essentially of a liquid mixture of isomers of tetrachlor benzyl cyanide having a pour point of about  $-5^{\circ}$  C., a viscosity of about 160 seconds at  $37.8^{\circ}$  C., and boiling in the range of about 220 to  $250^{\circ}$  C. at a pressure of about 25 mm. of mercury.
9. In an electric device, a dielectric and insulating composition consisting preponderantly of a liquid mixture of halogenated aromatic nitrile isomers, said composition containing halogen in an amount at least chemically equivalent to the hydrogen content thereof, being substantially non-inflammable and being capable of absorbing hydrogen halide.

FRANK M. CLARK.

20